

Aug. 2, 1932.

K. K. LEDIG

1,869,817

METHOD OF MAKING DENTAL PINS

Filed Aug. 9, 1929

Fig. 1.



Fig. 2.



Kurt K. Ledig  
INVENTOR  
BY  
Frank C. Fischer  
ATTORNEY

## UNITED STATES PATENT OFFICE

KURT K. LEDIG, OF NEWARK, NEW JERSEY, ASSIGNOR TO AMERICAN PLATINUM WORKS, OF NEWARK, NEW JERSEY, A CORPORATION OF NEW JERSEY

## METHOD OF MAKING DENTAL PINS

Application filed August 9, 1929. Serial No. 384,741.

This invention relates to dental pins used for holding teeth to gold or similar plates, and more particularly to a method of making such pins.

Dental pins of the type herein disclosed are necessarily small, seldom exceeding  $\frac{1}{4}$ " in length and  $\frac{1}{2}$ " in diameter, and due to their size, they have heretofore been cut from nickel wire upon which gold has been deposited by plating or rolling. However, pins made in accordance with such a method are objectionable as the points at which each pin is cut from the wire is not covered with gold with the result that small nickel surfaces are exposed to the corroding action of mouth acids.

It is an object of this invention to provide a method of making a dental pin by which no nickel surfaces are exposed to the corroding and dangerous action of mouth acids.

This and other objects are accomplished by the novel treatment of the metals employed as hereinafter described and claimed. In order to assist in the explanation of the method, the accompanying drawing is provided, in which:

Figure 1 is a sectional view of a dental pin made in accordance with my invention whereby the nickel base is completely covered so that no nickel surfaces are exposed.

Figure 2 is a sectional view showing the manner in which nickel surfaces are exposed on pins made in accordance with methods heretofore employed.

Referring to the drawing, in Figure 2, is shown a dental pin made in accordance with heretofore well known methods, in which a nickel base is covered with a gold plate 4.

The pin is cut from nickel wire upon which the gold has been deposited by plating or rolling, and as is shown in the drawing, the points at which the wire is cut leave on each pin, at the top and at the bottom, the areas 5 and 6, which are not covered by the gold

plate. The areas 5 and 6, being of nickel base 3, are attacked by the mouth acids.

In practicing my invention, the pins are first cut from a nickel wire and then plated with gold to produce a pin such as shown in Figure 1, having a base 7 of nickel, completely covered with a gold plate 8, and then the gold covered nickel base is heated in an electric furnace in proximity to a suitable reducing agent, such as charcoal, and the temperature of the furnace is raised to approximately 750 degrees centigrade, or at other temperatures depending upon the plating material employed, the temperature of the furnace being below the melting temperatures of the metals used.

The pin is allowed to remain in the furnace for approximately twenty minutes until the gold has been thoroughly diffused with the nickel base, so that an effective alloy is produced, at the junction of the nickel base and the gold plate.

While in the electric furnace under heat, the nickel base is protected from oxidation by the reducing agent, the latter also serving to destroy any minute coating of oxides which may be upon the surface of the base.

It should be noted that other reducing means besides charcoal and the electric furnace may be employed; for example, a diffusion of the plate into the metal of the pin may be accomplished by heating them in hydrogen gas. If the nickel bases are already free from oxide when placed into the furnace, a diffusion of the gold into the metal of the pin may be accomplished in a vacuum or in any inert gas, the essential point being the prevention of oxidation during the heating process.

A dental pin made in accordance with my method will have a metallic base completely covered with a gold plate firmly adhering thereto, and presenting no surfaces of the base metal exposed to the destructive acids of the mouth.

From the above description it will be seen that I have provided an effective and simple method of making satisfactory dental pins which are not effected by the mouth acids.

Having thus described my invention, what I claim as new and desire to secure by Letters Patent, is:

The method of making a dental pin having a nickel base, comprising plating the pin with 10 gold then heating the plated pin in a furnace containing charcoal at a temperature below the melting points of the metals used, to cause a diffusion of the gold plate with the nickel base, the gold plate completely covering the 15 pin.

This specification signed this 24th day of July, 1929.

KURT K. LEDIG.

20

25

30

35

40

45

50

55

60

65